# EUROPEAN PATENT SPECIFICATION

(11) **EP 0 948 584 B1**
(45) Date of publication and mention of the grant of the patent: **12.09.2001**
(21) Application number: 97911373.5
(22) Date of filing: 11.11.1997
(51) Int. Cl.: C10L 1/06, C10L 1/02

(54) **FUEL COMPOSITION**
BRENNSTOFFZUSAMMENSETZUNG
COMPOSITIONS COMBUSTIBLES

(30) Priority: 18.11.1996 GB 9623934
(43) Date of publication of application: 13.10.1999
(73) Proprietor: BP OIL INTERNATIONAL LIMITED, London EC2M 7BA (GB)
(72) Inventor: CLARK, Alisdair, Quentin, Hants GU12 6LS (GB)
(74) Representative: Hymers, Ronald Robson
(86) International application number: GB9703084
(87) International publication number: WO9822556

(56) References cited:
- GB-A- 2 106 933
- US-A- 4 633 028
- DATABASE WPI Section Ch, Week 9622 Derwent Publications Ltd., London, GB; Class H06, AN 96-220407 XP002054753 & RU 2 044 032 C (INTERAVIAGAZ STOCK CO)

## Description

The present invention relates to fuel compositions and in particular aviation gasolines possessing a high octane number suitable for use in piston-driven aircraft.

If a gasoline engine is run on a fuel which has an octane number lower than the minimum requirement for the engine, knocking will occur. Straight run gasoline has a low motor octane number but may be boosted to the required motor octane number of 82-88 for automotive use by the addition of octane boosters such as tetraethyl lead either alone or with refinery components such as reformate, alkylate, cracked spirit or chemical streams such as toluene, xylene, methyl tertiary butyl ether or ethanol. Aircraft piston-driven engines operate under extreme conditions to deliver the desired power e.g. high compression ratios. Due to the severity of the conditions e.g. with turbo charging or super charging the engine, aviation piston-driven engines require fuel of a minimum octane level higher than that for automotive internal combustion gasoline engines, in particular at least 98-100. The base fuel of an aviation gasoline has a motor octane number of 90-93. To boost the motor octane number sufficiently to the required level, tetraethyl lead is added to the aviation base fuel. The fuel may contain the organolead and also other octane boosters, such as those described above. Industrial and Engineering Chemistry Vol. 36 No. 12 p1079-1084 dated 1944 describes the use of triptane (2,2,3-trimethylbutane) in combination with tetraethyl lead in aviation gasoline. However, the presence of tetraethyl lead is the key to achieving high octane quality in aviation gasolines.

In modern day formulations tetraethyl lead is always used to boost the octane quality of the aviation gasoline to the desired level. However due to environmental concerns of the effect of lead and its compounds attempts are being made to find an alternative to the use of tetraethyl lead in aviation gasoline. Conventional octane boosters such as ethers, aromatics, such as toluene, and non-lead metal compounds can boost the motor octane number of unleaded motor gasoline sufficiently high enough to achieve the desired value but they do not boost the motor octane number of an unleaded aviation gasoline sufficiently high enough to ensure satisfactory performance or suffer from other significant technical limitations.

US 5470358 describes the use of aromatic amines to boost the motor octane number of unleaded aviation gasoline to at least 98 but many aromatic amines are known to be toxic. They have high boiling points, no supercharge properties and high freezing points; they are also prone to produce gums.

There remains a need for an unleaded aviation gasoline of sufficiently high octane number suitable for use in piston driven aircraft

According to the present invention there is provided an unleaded aviation fuel composition, having a Motor Octane Number of at least 98, and usually a final Boiling Point of less than 170°C, and preferably a Reid Vapour Pressure at 37.8°C of between 38-60 kPascals,
which comprises:
component (a) at least one hydrocarbon having the following formula I

R-CH₂-CH(CH₃)-C(CH₃)₂-CH₃ I

wherein R is hydrogen or methyl
and component (b) at least one saturated liquid aliphatic hydrocarbon having 4 to 10 in particular 5 or 6 carbon atoms optionally with at least one other saturated liquid aliphatic hydrocarbon having from 5 to 10 carbon atoms
wherein at least 30% by volume of the total composition is a hydrocarbon of formula I.

If R is hydrogen the hydrocarbon is triptane. If R is methyl the hydrocarbon is 2,2,3 trimethylpentane. Especially preferred is triptane. Triptane and 2,2,3 trimethylpentane may be used individually or in combination with each other, for example, in a weight ratio of 10:90 - 90:10, preferably, 30:70 - 70:30.

The composition may comprise apart from a component (I), the hydrocarbon of formula I, a component (II) which is at least one of the known octane boosters described above especially an oxygenate octane booster, usually an ether, usually of Motor Octane Number of at least 96-105 e.g. 98-103. The ether octane booster is usually a dialkyl ether, in particular an asymmetric one, preferably wherein each alkyl has 1-6 carbons, in particular one alkyl being a branched chain alkyl of 3-6 carbons in particular a tertiary alkyl especially of 4-6 carbons such as tert-butyl or tert-amyl, and with the other alkyl being of 1-6 e.g. 1-3 carbons, especially linear, such as methyl or ethyl. Examples of component (II) include methyl tertiary butyl ether, ethyl tertiary butyl ether and methyl tertiary amyl ether. The oxygenate may also be an alcohol of 1-6 carbons e.g. ethanol.

At least one component (I) may be present together with at least one component (II) in a combination. The combination may be, for example, triptane together with methyl tertiary butyl ether. The combination may be in a volume ratio of 40:60 to 99:1 e.g. 50:50 to 90 : 10, preferably 60:40 to 85:15. The volume percentage of ether may be up to 30% of the total composition e.g. 1-30%, such as 1-15% or 5-25%.

The motor octane number of the aviation gasoline of the invention is at least 98, for example 98-103, preferably 99 to 102. Motor Octane Numbers are determined according to ASTM D 2700-92. The hydrocarbons of formula I may also, especially when present in amount of at least 30% by volume, be used to provide gasolines of the invention with a Performance Number (according to ASTM D909) of at least 130 e.g. 130-170.

Triptane or 2,2,3 trimethylpentane may be used in a purity of at least 95% but is preferably used as part of a hydrocarbon mixture obtained, via distillation of a cracked residue, which is an atmospheric or vacuum residue from crude oil distillation, to give a C₄ fraction containing olefin and hydrocarbon, alkylation to produce a C₄₋₉ especially a C₆₋₉ fraction which is distilled to give a predominantly C₈ fraction, which usually contains trimethyl pentanes including 223 trimethyl pentane and/or 233 trimethyl pentane. To produce triptane this fraction can be demethylated to give a crude product comprising at least 5% of triptane, which can be distilled to increase the triptane content in the mixture; such a distillate may comprise at least 10% or 20% of triptane and 2,2,3 trimethylpentane but especially at least 50% e.g. 50-90% the rest being predominantly of other aliphatic C7 and C8 hydrocarbons e.g. in amount 10-50% by volume. Alternatively triptane and 2,2,3 trimethylpentane may be used in any commercially available form.

The invention will be further described with triptane exemplifying the compound of formula I but 2,2,3 trimethylpentane may be used instead or as well.

The amount of the hydrocarbon of Formula I alone or with component II may be present in the composition in an effective amount to boost the Motor Octane Number to at least 98 and may be in a percentage of from 35-92%, preferably 60-90%, especially 70-90% by volume, based on the total volume of the composition. In particular the compound of formula I is usually in the composition in a percentage of 5-90%, 10-80%, 20-60% more especially 30-50% by volume, based on the total composition, though amounts of the compound of formula I of 10-45% are also very valuable; preferred are 20-90% or 40-90% or 50-90% by volume.

The composition also comprises a component (b). Component (b) is at least one saturated aliphatic liquid hydrocarbon of 4 to 10 preferably 5 to 8 in particular 5 or 6 carbon atoms, alone or with at least one saturated aliphatic liquid hydrocarbon (different from component(a)) having from 4 to 10 carbons in particular 5 to 10 carbon atoms, preferably 5 to 8 carbon atoms, especially in combination with one of 4 carbons. Component (b) may comprise a component (III) which is more volatile and has a lower boiling point than component (a) in particular one boiling at least 30°C such as 30-60°C below that of triptane at atmospheric pressure, and especially is itself of Motor Octane Number greater than 88 in particular at least 90 e.g. 88-93 or 90-92. Examples of component (III) include alkanes of 5 carbons in particular iso-pentane, which may be substantially pure or a crude hydrocarbon fraction from alkylate or isomerate containing at least 30% e.g. 30-80% such as 50-70%, the main contaminant being up to 40% mono methyl pentanes and up to 50% dimethyl butanes. Component (III) of boiling point 30-60°C less than that of triptane may be used as sole component (III) but may be mixed with an alkane of boiling point 60-100°C less than that of triptane e.g. n and/or iso butane in blends of 99.5:0.5 to 70:30, e.g. 88:12 to 75:25. Iso-pentane alone or mixed with n-butane is preferred, especially in the above proportions, and in particular with a volume amount of butane in the composition of up to 3.5% e.g. 1-3.5% or 2-3.5%.

Component (b) may also comprise a component (IV) having a boiling point higher than component (a) preferably one boiling at least 20°C more than the compound of formula I e.g. triptane such as 20-60°C more than triptane but less than 170°C and usually is of Motor Octane Number of at least 92 e.g. 92-100; such components (IV) are usually alkanes of 7-10 carbons especially 7 or 8 carbons, and in particular have at least one branch in their alkyl chain, in particular 1-3 branches, and preferably on an internal carbon atom and especially contain at least one -C(CH₃)₂- group. An example of component (IV) is iso-octane.

Component (b) may be a combination of at least one component (III) together with at least one component (IV). The combination may be, for example, butane or isopentane together with iso-octane, and the combination may be in a volume ratio of 10 : 90 to 90 : 10, preferably 10:50 to 50:90, especially 15:85 to 35:65, in particular with butane or especially isopentane together with iso-octane. Especially preferred is the combination of isopentane together with iso-octane, in particular, in the above proportions, and optionally butane.

In another preferred embodiment, triptane and isopentane and optionally n-butane are present in the composition of the invention with 80-90% triptane and in particular in relative volume ratios of 80-90:10-15:0-3.5.

In a preferred embodiment of this invention component (a) is 2,2,3 trimethylbutane and component (b) is isopentane in combination with iso-octane, preferably in relative volume ratios of 10-80 : 5-25 : 10:80 in particular 30-50 : 5-25 : 35-60 or 15-45 : 10-18 : 45-75 or 60-80 : 10-18 : 10-25. Especially the composition contains 30-80% of triptane and the isopentane and iso-octane are in a volume ratio of 35-15 : 65-85.

In a further preferred embodiment of this invention the composition comprises component (a) as 2,2,3 trimethylbutane, methyl tertiary butyl ether and component (b) as isopentane in combination with n-butane, preferably in relative volume ratios of 50-90 : 5-30 : 10-15 : 0.1-3.5 in particular 50-80 : 10-25 : 10-15 : 0.1-3.5.

If desired the composition may comprise an aromatic liquid hydrocarbon of 6-9 e.g. 6-8 or 7-9 carbons, such as xylene or a trimethyl benzene, preferably but toluene, in particular in amounts of up to 30% by volume of the total composition e.g. 1-30% or 5-15%. In this case a preferred embodiment is a composition that may thus contain 50-95% e.g. 50-80% triptane, 5-25% e.g. 10-25% component (b) e.g. isopentane and 5-30%, for example toluene. The benzene content of the composition is preferably less than 0.1% by volume.

In another preferred embodiment the composition may comprise both the aromatic hydrocarbon and the ether. In this case a preferred composition may comprise 45-80% triptane 5-30% ether (with a preferred total of both of 70-85%), 10-25% component (b) (III) e.g. iso-pentane (optionally containing butane) and 5-20% toluene, all by volume.

The compositions may also comprise 10-90% e.g. 25-85%, 35-80%, or 35-90% by volume of triptane, 5-75% e.g. 8-55% by volume of a mixture predominantly of iso C₇ and iso C₈ hydrocarbons, but usually with small amounts of iso C₆ and iso C₉ hydrocarbons and 5-40% e.g. 8-40% or 5-35% or 8-25% by volume isopentane. The triptane and mixture may be obtained as a distillation fraction obtained by the processing of crude oil and subsequent reactions as described above.

The unleaded aviation gasoline composition of the invention usually has a calorific value (also called Specific Energy) of at least 42MJ/kg (18075 BTU/lb) e.g. at least 43.5MJ/kg (18720 BTU/lb) such as 42-46 or 43.5-45MJ/kg. The gasoline usually has a boiling range (ASTM D86) of 25- 170°C and is usually such that at 75°C 10-40% by volume is evaporated, at 105°C a minimum of 50% is evaporated, at 135°C a minimum of 90% is evaporated; the final boiling point is usually not more than 170°C preferably 80-130°C. The gasoline usually has a maximum freezing point of -60°C in particular -40°C. The Reid Vapour Pressure of the gasoline at 37.8°C measured according to ASTM D323 is usually 30-60kPa preferably 38-60 e.g. 38-55 or especially 38-49 or 45-55kPa.

The composition of the invention may contain at least one aviation gasoline additive, for example as listed in ASTM D-910 or DEF-STAN 91-90; examples of additives are anti-oxidants, corrosion inhibitors, anti-icing additives e.g. glycol ethers or alcohols and anti-static additives, especially antioxidants such as one or more hindered phenols; in particular the additives may be present in the composition in amounts of 0.1-100ppm e.g. 1-20ppm, usually of an antioxidant especially one or more hindered phenols. A coloured dye may also be present to differentiate the aviation gasoline from other grades of fuel.

The compositions of the invention are unleaded and have reduced toxicity, and are suitable for use in aviation gasoline for piston engine aircraft. Aromatic amines e.g. m-toluidine are usually substantially absent.

The invention will be illustrated by way of the following Examples

### Example 1

An unleaded aviation gasoline was made by mixing 2,2,3 trimethylbutane of 99% purity with iso-pentane and iso-octane to give a composition consisting of 2,2,3 trimethylbutane 40%, isopentane 12%, and iso-octane 48% expressed in volume percentages of the total gasoline.

The motor octane number (MON) of the gasoline was 99.9 as determined by ASTM D2700-92 and the Reid Vapour Pressure was 33kPa.

### Example 2

An unleaded aviation gasoline contained the gasoline of Ex.1 with 8mg/l of a mixture of 75% 2,6-ditertiary, butyl phenol and 25% tertiary and tri tertiary, butyl phenols, as antioxidant.

### Example 3

An unleaded aviation gasoline was made from a crude triptane fraction. A cracked residue from the distillation of crude oil was distilled to give a C₄ fraction containing olefin and saturates. The fraction was alkylated (i.e. self reacted) to form a crude C₈ saturate which was distilled to give a fraction boiling 95-120°C, which contained 223 and 233 trimethyl pentane. This fraction was demethylated by reduction to give a first fraction containing about 17% triptane and 83% iso C₆-C₉ with a majority of iso C₇ and iso C₈ hydrocarbons. This first fraction was redistilled to produce a second fraction of 87% triptane and 13% iso C₇ and C₈.

90 parts by volume of this second fraction was mixed with 10 parts of isopentane to give an unleaded aviation gasoline of MON value 99.1. Addition of 8mg/l of the phenol mixture of Ex.2 gave an oxidation stabilized unleaded aviation gasoline fuel.

### Example 4

The process of Example 3 was repeated with the first fraction containing the 17% triptane redistilled to give a third fraction containing 37% triptane and 63% iso C₇ and C₈. 82 parts by volume of this third fraction were mixed with 18 parts of isopentane to give an unleaded aviation gasoline of MON value 98.0. Addition of the phenol mixture as in Ex.3 gave an oxidation stabilised aviation gasoline fuel.

### Examples 5-9

In these Examples 2,2,3 trimethylbutane (triptane) 99% purity was mixed with iso-pentane and butane, and optionally toluene and/or methyl tertiary butyl ether, to produce a series of gasoline blends, for making unleaded aviation gasolines.

The formulated gasolines were made by mixing each blend with a phenolic antioxidant 55% minimum 2,4 dimethyl-6-tertiary butyl phenol 15% minimum 4 methyl-2, 6-ditertiary-butyl phenol with the remainder as a mixture of monomethyl and dimethyl-tertiary butyl phenols (DEF STAN 91-90 RDE/A/610)

In each case the gasolines were tested for Motor Octane Number, and their Reid Vapour Pressure at 37.8°C and their calorific value, and their distillation properties and freezing point. In addition for Example 10 the Indicated Mean Effective Pressure (IMEP) was determined (according to ASTM D909) to give the Supercharge Performance Number. The results are shown in table 1.

**Table 1**

| **Example** | **5** | **6** | **7** | **8** | **9** |
|---|---|---|---|---|---|
| Composition % v/v | | | | | |
| Triptane | 85.0 | 73.0 | 53.0 | 87.8 | 87.0 |
| Isopentane | 12.0 | 14.0 | 14.0 | 12.0 | 11.8 |
| Butane | 3.0 | 3.0 | 3.0 | 0.2 | 1.2 |
| Toluene | - | 10.0 | 10.0 | - | - |
| MTBE | - | - | 20.0 | - | - |
| Antioxidant mg/l | 15 | 15 | 24 | 17 | 15 |
| | | | | | |

| Distillation °C | | | | | |
|---|---|---|---|---|---|
| Initial Boiling Point | 43.0 | 41.0 | 36.5 | 47.5 | 46.5 |
| T10% | 63.5 | 63.5 | 57.0 | 68.0 | 67.0 |
| T40% | 77.0 | 79.0 | 69.9 | 76.5 | 77.0 |
| T50% | 78.5 | 81.5 | 73.8 | 78.5 | 79.0 |
| T90% | 80.5 | 87.5 | 88.4 | 80.5 | 81.0 |
| Final Boiling Point | 115.0 | 116.0 | 107.7 | 80.5 | 90.0 |
| | | | | | |
| Reid Vapour Pressure kPa | 51.3 | 52.5 | 58.3 | 40.4 | 46.3 |
| | | | | | |
| MON | 99.8 | 98.3 | 98.0 | 99.7 | 99.8 |
| | | | | | |
| Freezing point °C | -54 | <-80 | <-80 | -49 | -51.5 |
| | | | | | |
| Supercharge (IMEP) | - | - | - | - | >160 |
| | | | | | |
| Specific energy MJ/kg | 44.5 | 44.1 | 42.1 | 44.5 | 44.5 |

T 10% means the temperature at which 10% by volume of the composition has distilled.

## Claims

1. An unleaded aviation fuel composition, having a Motor Octane Number of at least 98, and having a final boiling point of less than 170°C which comprises:
component (a) comprising at least one hydrocarbon having the following formula I
R-CH₂-CH(CH₃)-C(CH₃)₂-CH₃ (I)
wherein R is hydrogen or methyl
and component
(b) at least one saturated liquid aliphatic hydrocarbon having 5 or 6 carbon atoms
wherein at least 30% by volume of the total composition is a hydrocarbon of formula I.

2. A composition according to Claim 1 wherein the hydrocarbon of formula I is triptane.

3. A composition according to Claim 1 or 2 having a Reid Vapour Pressure at 37.8°C of 38 - 60 kPascals.

4. A composition according to Claim 3 with a Reid Vapour Pressure of 38-49 kPascals.

5. A composition according to anyone of the preceding Claims wherein component (b) comprises a component (III) which is more volatile and has a lower boiling point than triptane.

6. A composition according to Claim 5 wherein component (III) has a Motor Octane Number greater than 88.

7. A composition according to either of Claims 5 or 6 wherein component (III) comprises iso-pentane.

8. A composition according to Claim 7 wherein the fuel composition comprises 5-40% by volume of iso-pentane.

9. A blend according to claim 8 which comprises 5-25% by volume ofisopentane.

10. A composition according to any one of Claims 7-9 wherein component (III) comprises butane and iso-pentane.

11. A composition according to anyone of the preceding Claims wherein the fuel composition comprises 0.1-3.0 % by volume of n-butane.

12. A composition according to any one of the Claims 5-11 wherein component (b) comprises in addition to component (III) a component (IV) having a boiling point higher than triptane but less than 170°C.

13. A composition according to Claim 12 wherein component (IV) has a Motor Octane Number of at least 92.

14. A composition according to either of the preceding Claims 12 or 13 wherein component (IV) is iso-octane.

15. A composition according to anyone of the preceding Claims wherein the composition comprises up to 30% by volume of an aromatic liquid hydrocarbon of 6-8 carbons.

16. A composition according to Claim 15 wherein the composition comprises 5-30% by volume of toluene.

17. A composition according to any one of the preceding claims which comprises as component (I) said hydrocarbon having the formula I and a component (II) an oxygenate octane booster.

18. A composition according to Claim 17 wherein the component (II) is an ether.

19. A composition according to Claim 18 wherein the ether is methyl tertiary butyl ether.

20. A composition according to anyone of the preceding Claims wherein 35-92% by volume of the total composition is the combined volume of the hydrocarbon of formula I and methyl tertiary butyl ether (if present).

21. A composition according to any one of Claims 1-14 which comprises 80-90% of triptane, with isopentane and optionally butane.

22. A composition according to any one of Claims 1-14 which comprises 30-80% of triptane, and also III isopentane and IV iso-octane, the volume ratio of III to IV being 35-15:65-85.

23. A composition according to Claim 16 which comprises 50-90% triptane, 5-25% isopentane and 5-30% toluene.

24. A composition according to Claim 23 which comprises 0-15% methyl tertiary butyl ether.

25. A composition according to anyone of the preceding Claims which has a calorific value of at least 42MJ/kg.

26. A composition according to Claim 25 which has a calorific value of at least 43.5MJ/kg.

27. A composition according to anyone of the preceding Claims wherein the Performance Number for supercharging is at least 130.

28. An unleaded aviation fuel having a Motor Octane Number of at least 98, and having a final boiling point of less than 170°C which comprises:
component (a) comprising at least one hydrocarbon having the following formula I
R-CH₂-CH(CH₃)-C(CH₃)₂-CH₃ (I)
wherein R is hydrogen or methyl
and component
(b) at least one saturated liquid aliphatic hydrocarbon having 5 or 6 carbon atoms wherein at least 20% by volume of the total composition is a hydrocarbon of formula I, together with at least one aviation gasoline additive selected from antioxidants, corrosion inhibitors, anti-icing additives and anti-static additives.

29. A fuel according to Claim 28 wherein the antioxidant is one or more hindered phenols.

30. Use of the hydrocarbon of formula I as an octane booster in an unleaded aviation gasoline to give a composition or fuel as claimed in any of the preceding claims.

31. The use of an unleaded aviation fuel according to Claim 28 or 29 in an aircraft piston driven engine.

## Patentansprüche

1. Unverbleite Flugzeugkraftstoff-Zusammensetzung mit einer Motoroctanzahl von mindestens 98 und mit einem Endsiedepunkt von weniger als 170°C, welche umfasst:
Komponente (a), umfassend mindestens einen Kohlenwasserstoff der nachstehenden Formel I
R-CH₂-CH(CH₃)-C(CH₃)₂-CH₃ (I)
worin R Wasserstoff oder Methyl darstellt,
und Komponente (b) mindestens einen gesättigten flüssigen, aliphatischen Kohlenwasserstoff mit 5 oder 6 Kohlenstoffatomen, wobei mindestens 30 Volumenprozent der gesamten Zusammensetzung ein Kohlenwasserstoff der Formel I sind.

2. Zusammensetzung nach Anspruch 1, worin der Kohlenwasserstoff der Formel I Triptan ist.

3. Zusammensetzung nach Anspruch 1 oder 2 mit einem Reid-Dampfdruck bei 37,8°C von 38 - 60 kPa.

4. Zusammensetzung nach Anspruch 3, mit einem Reid-Dampfdruck von 38-49 kPa.

5. Zusammensetzung nach einem der vorangehenden Ansprüche, wobei Komponente (b) eine Komponente (III) umfasst, die flüchtiger ist und einen niedrigeren Siedepunkt als Triptan aufweist.

6. Zusammensetzung nach Anspruch 5, wobei Komponente (III) eine Motoroctanzahl größer als 88 aufweist.

7. Zusammensetzung nach einem der Ansprüche 5 oder 6, wobei Komponente (III) Isopentan umfasst.

8. Zusammensetzung nach Anspruch 7, wobei die Kraftstoffzusammensetzung 5-40 Volumenprozent Isopentan umfasst.

9. Gemisch nach Anspruch 8, das 5-25 Volumenprozent Isopentan umfasst.

10. Zusammensetzung nach einem der Ansprüche 7-9, wobei Komponente (III) Butan und Isopentan umfasst.

11. Zusammensetzung nach einem der vorangehenden Ansprüche, wobei die Kraftstoffzusammensetzung 0,1-3,0 Volumenprozent n-Butan umfasst.

12. Zusammensetzung nach einem der Ansprüche 5-11, wobei Komponente (b) zusätzlich zu Komponente (III) eine Komponente (IV) mit einem Siedepunkt höher als Triptan, jedoch unterhalb 170°C umfasst.

13. Zusammensetzung nach Anspruch 12, wobei Komponente (IV) eine Motoroctanzahl von mindestens 92 aufweist.

14. Zusammensetzung nach einem der vorangehenden Ansprüche 12 oder 13, wobei Komponente (IV) Isooctan ist.

15. Zusammensetzung nach einem der vorangehenden Ansprüche, wobei die Zusammensetzung bis zu 30 Volumenprozent eines aromatischen flüssigen Kohlenwasserstoffs mit 6-8 Kohlenstoffatomen umfasst.

16. Zusammensetzung nach Anspruch 15, wobei die Zusammensetzung 5-30 Volumenprozent Toluol umfasst.

17. Zusammensetzung nach einem der vorangehenden Ansprüche, die als Komponente (I) den Kohlenwasserstoff mit der Formel I und eine Komponente (II), einen Oxygenatoctanverbesserer, umfasst.

18. Zusammensetzung nach Anspruch 17, worin die Komponente (II) ein Ether ist.

19. Zusammensetzung nach Anspruch 18, worin der Ether Methyl-tert-butylether ist.

20. Zusammensetzung nach einem der vorangehenden Ansprüche, wobei 35-92 Volumenprozent der gesamten Zusammensetzung das vereinigte Volumen von dem Kohlenwasserstoff der Formel I und Methyl-tert-butylether (falls vorliegend) ist.

21. Zusammensetzung nach einem der Ansprüche 1-14, die 80-90% Triptan mit Isopentan und gegebenenfalls Butan umfasst.

22. Zusammensetzung nach einem der Ansprüche 1-14, die 30-80% Triptan und auch III Isopentan und IV Isooctan umfasst, wobei das Volumenverhältnis von III zu IV 35-15:65-85 ist.

23. Zusammensetzung nach Anspruch 16, die 50-90% Triptan, 5-25% Isopentan und 5-30% Toluol umfasst.

24. Zusammensetzung nach Anspruch 23, die 0-15% Methyl-tert-butylether umfasst.

25. Zusammensetzung nach einem der vorangehenden Ansprüche, die einen Wärmewert von mindestens 42 MJ/kg aufweist.

26. Zusammensetzung nach Anspruch 25, die einen Wärmewert von mindestens 43,5 MJ/kg aufweist.

27. Zusammensetzung nach einem der vorangehenden Ansprüche, wobei die Leistungszahl zum Vorverdichten mindestens 130 ist.

28. Unverbleiter Flugzeugkraftstoff mit einer Motoroctanzahl von mindestens 98 und mit einem Endsiedepunkt von weniger als 170°C, der umfasst:
Komponente (a), umfassend mindestens einen Kohlenwasserstoff der nachstehenden Formel I
R-CH₂-CH(CH₃)-C(CH₃)₂-CH₃ (I)
worin R Wasserstoff oder Methyl darstellt,
und Komponente (b) mindestens einen gesättigten flüssigen, aliphatischen Kohlenwasserstoff mit 5 oder 6 Kohlenstoffatomen, wobei mindestens 20 Volumenprozent der gesamten Zusammensetzung ein Kohlenwasserstoff der Formel I sind, zusammen mit mindestens einem Flugzeugbenzin-Additiv, ausgewählt aus Antioxidantien, Korrosionsinhibitoren, Antivereisungsadditiven und antistatischen Additiven.

29. Kraftstoff nach Anspruch 28, wobei das Antioxidans ein oder mehrere gehinderte Phenole sind.

30. Verwendung des Kohlenwasserstoffs der Formel I als ein Octanverbesserer in einem unverbleiten Flugzeugbenzin unter Gewinnung einer Zusammensetzung oder eines Kraftstoffs nach einem der vorangehenden Ansprüche.

31. Verwendung eines unverbleiten Flugzeugkraftstoffs nach Anspruch 28 oder 29 in einem Flugzeugkolbenmotor.

## Revendications

1. Composition de combustible aviation sans plomb, ayant un indice d'octane moteur d'au moins 98, et ayant un point d'ébullition final inférieur à 170°C, qui comprend :
un composant (a) comprenant au moins un hydrocarbure ayant la formule I suivante
R-CH₂-CH(CH₃)-C(CH₃)₂-CH₃ (I)
dans laquelle R est l'hydrogène ou le méthyle
et un composant (b) : au moins un hydrocarbure aliphatique liquide saturé ayant 5 ou 6 atomes de carbone
dans laquelle au moins 30% en volume de la composition totale est un hydrocarbure de la formule I.

2. Composition selon la revendication 1, dans laquelle l'hydrocarbure de la formule I est le triptane.

3. Composition selon la revendication 1 ou 2, ayant une tension de vapeur Reid à 37,8°C de 38 à 60 kPascals.

4. Composition selon la revendication 3, avec une tension de vapeur Reid de 38 à 49 kPascals.

5. Composition selon l'une quelconque des revendications précédentes, dans laquelle le composant (b) comprend un composant (III) qui est plus volatil et a un point d'ébullition inférieur à celui du triptane.

6. Composition selon la revendication 5, dans laquelle le composant (III) a un indice d'octane moteur supérieur à 88.

7. Composition selon l'une ou l'autre des revendications 5 ou 6, dans laquelle le composant (III) comprend de l'isopentane.

8. Composition selon la revendication 7, dans laquelle la composition de combustible comprend de 5 à 40% en volume d'isopentane.

9. Mélange selon la revendication 8, qui comprend de 5 à 25% en volume d'isopentane.

10. Composition selon l'une quelconque des revendications 7 à 9, dans laquelle le composant (III) comprend du butane et de l'isopentane.

11. Composition selon l'une quelconque des revendications précédentes, dans laquelle la composition combustible comprend de 0,1 à 3,0% en volume de n-butane.

12. Composition selon l'une quelconque des revendications 5 à 11, dans laquelle le composant (b) comprend en plus du composant (III) un composant (IV) ayant un point d'ébullition supérieur à celui du triptane mais inférieur à 170°C.

13. Composition selon la revendication 12, dans laquelle le composant (IV) a un indice d'octane moteur d'au moins 92.

14. Composition selon l'une ou l'autre des revendications précédentes 12 ou 13, dans laquelle le composant (IV) est l'isooctane.

15. Composition selon l'une quelconque des revendications précédentes, dans laquelle la composition comprend jusqu'à 30% en volume d'un hydrocarbure liquide aromatique ayant de 6 à 8 carbones.

16. Composition selon la revendication 15, dans laquelle la composition comprend de 5 à 30% en volume de toluène.

17. Composition selon l'une quelconque des revendications précédentes, qui comprend comme composant (I) ledit hydrocarbure ayant la formule I et un composant (II), un agent d'élévation de l'indice d'octane oxygéné.

18. Composition selon la revendication 17, dans laquelle le composant (II) est un éther.

19. Composition selon la revendication 18, dans laquelle l'éther et l'éther méthylterbutylique.

20. Composition selon l'une quelconque des revendications précédentes, dans laquelle de 35 à 92% en volume de la composition totale est constitué par le volume combiné de l'hydrocarbure de la formule I et de l'éther méthylterbutylique (s'il est présent).

21. Composition selon l'une quelconque des revendications 1 à 14, qui comprend de 80 à 90% de triptane, avec de l'isopentane et, facultativement, du butane.

22. Composition selon l'une quelconque des revendications 1 à 14, qui comprend de 30 à 80% de triptane, ainsi que de l'isopentane III et de l'isooctane IV, le rapport en volume de III sur IV étant de 35-15/65-85.

23. Composition selon la revendication 16, qui comprend de 50 à 90% de triptane, de 5 à 25% d'isopentane et de 5 à 30% de toluène.

24. Composition selon la revendication 23, qui comprend de 0 à 15% d'éther méthylterbutylique.

25. Composition selon l'une quelconque des revendications précédentes, qui a un pouvoir calorifique d'au moins 42 MJ/kg.

26. Composition selon la revendication 25, qui a un pouvoir calorifique d'au moins 43,5 MJ/kg.

27. Composition selon l'une quelconque des revendications précédentes, dans laquelle l'indice de performance pour la suralimentation est d'au moins 130.

28. Combustible aviation sans plomb, ayant un indicè d'octane moteur d'au moins 98, et ayant un point d'ébullition final inférieur à 170°C, qui comprend
un composant (a) comprenant au moins un hydrocarbure ayant la formule I suivante
R-CH₂-CH(CH₃)-C(CH₃)₂-CH₃ (I)
dans laquelle R est l'hydrogène ou le méthyle
et un composant (b) : au moins un hydrocarbure aliphatique liquide saturé ayant 5 ou 6 atomes de carbone dans laquelle au moins 20% en volume de la composition totale est un hydrocarbure de la formule I, avec au moins un additif pour essence d'aviation choisi parmi les antioxydants, les inhibiteurs de corrosion, les additifs antigivrage et les additifs antistatiques.

29. Combustible selon la revendication 28, dans lequel l'antioxydant est un ou plusieurs phénols encombrés.

30. Utilisation de l'hydrocarbure de la formule I en tant qu'agent d'élévation de l'indice d'octane dans une essence d'aviation sans plomb afin d'obtenir une composition ou carburant selon l'une quelconque des revendications précédentes.

31. Utilisation d'un combustible aviation sans plomb selon la revendication 28 ou 29 dans un moteur à pistons d'avion.
